

**United States Patent** [19]

Komamura et al.

[11] **Patent Number:** 4,650,748[45] **Date of Patent:** Mar. 17, 1987[54] **HEAT-DEVELOPABLE COLOR  
PHOTO-SENSITIVE MATERIAL**[75] Inventors: **Tawara Komamura, Hachioji;  
Hidenobu Ohya, Musashino, both of  
Japan**[73] Assignee: **Konishiroku Photo Industry Co., Ltd.,  
Japan**[21] Appl. No.: **812,728**[22] Filed: **Dec. 23, 1985**[30] **Foreign Application Priority Data**

Dec. 24, 1984 [JP] Japan ..... 59-272335

[51] Int. Cl.<sup>4</sup> ..... G03C 1/40; G03C 5/54  
[52] U.S. Cl. ..... 430/548; 430/203;  
430/226; 430/557

[58] Field of Search ..... 430/203, 226, 548, 557

[56]

**References Cited****U.S. PATENT DOCUMENTS**4,304,845 12/1981 Fujimatsu et al. ..... 430/557  
4,455,363 6/1984 Naito et al. ..... 430/548  
4,500,624 2/1985 Aono et al. ..... 430/203*Primary Examiner—Richard L. Schilling  
Attorney, Agent, or Firm—Finnegan, Henderson,  
Farabow, Garrett & Dunner*

[57]

**ABSTRACT**

A heat-developable color photo-sensitive material having a support. On the support, there is a photographic component layer containing at least a photo-sensitive silver halide, a reducing agent, a binder and a dye-providing material. At least one of the dye-providing materials in the photo-sensitive material is a polymer having a unit derived from a monomer represented by Formula I.

**12 Claims, No Drawings**

## HEAT-DEVELOPABLE COLOR PHOTO-SENSITIVE MATERIAL

### BACKGROUND OF THE INVENTION

This invention relates to a heat-developable color photo-sensitive material in which a color-image is produced by transferring a diffusible dye formed in a heat-development process, and more particularly to a heat-developable color photo-sensitive material containing a novel dye-providing material capable of producing a diffusible dye through a heat-development process.

Photographic method using a photo-sensitive silver halide has so far been known and that is superior to the other photographic methods in photo-sensitivity, gradation and image preservability and has most popularly been put into practice.

In this method, however, a wet-process has been applied to such a processing step as a developing, fixing or washing step. There have accordingly been many problems such as that it cannot help taking a lot of time and trouble and concerning about the influence of processing chemicals on the human body or about the chemical pollution of a processing room and an operator, and further taking care of industrial waste pollution. It has therefore been demanded to develop a photo-sensitive material capable of using a photo-sensitive material therein and being applied with a dry-process.

There have been made a number of proposals of the above-mentioned dry-processing photographic methods. Among them, a heat-developable photo-sensitive material capable of being developed by a heat-treatment has now become the object of public attention.

Concerning these heat-developable photo-sensitive materials the photo-sensitive materials each comprising an organic silver salt, a silver halide and a reducing agent are disclosed in, for example, Japanese Patent Examined Publication Nos. 4921/1968 and 4924/1968.

There have been the attempts to obtain color-images in a variety of methods through the improvements on the above-mentioned photo-sensitive materials.

For example, the heat-developable color photo-sensitive materials for forming color images through the reaction of couplers with the oxidants of an aromatic primary amine developing agent are disclosed in U.S. Pat. Nos. 3,531,286, 3,761,270, 3,764,328 and the like.

In Research Disclosure, Nos. 15,108 and 15,127, the heat-developable color photo-sensitive materials are disclosed to produce color images through the reaction of couplers with the oxidants of developing agent of a sulfonamidophenol derivative or a sulfonamidoaniline derivative. In these processes, however, a reduced silver image and a color image are produced simultaneously on an exposed area after heat-developed, and the color image is made turbid, that is a problem. As for the methods of solving such a problem, there are some methods such as that a silver image is removed in a liquid process or that dyes only are transferred to other layer such as an image receiving sheet having an image receiving layer, however, there is also a problem that it is not so easy to transfer the dyes only to the image receiving sheet with the discrimination thereof from the substances remaining unreacted.

Further, in Research Disclosure, No. 16,966, there discloses a heat-developable color photo-sensitive material in which an organic imino salt having dyes as the composition thereof is used so as to split off the imino group in an exposed area through a heat-development,

and a color image is produced on an image receiving layer in the form of a sheet of transfer-paper by making use of a solvent. In this process, however, there is a problem that it is impossible to obtain a sharp and clear color image because it is difficult to inhibit the splitting-off of the dyes in an area out of light.

Still further, in Japanese Patent O.P.I. Publication Nos. 105821/1977, 105822/1977 and 50328/1981; U.S. Pat. No. 4,235,957; Research Disclosure, Nos. 14,448, 15,227 and 18,137; and the like, there are disclosed the respective heat-developable color photo-sensitive materials in which a positive color image can be produced in a heat-sensitive silver dye bleach process. Wherein, 10 there are problems that an extra processing step and photographic component material are required, such as that some sheets containing an activator for accelerating the bleach of dyes are superposed together and are then heated, and that the obtained color image is gradually reduced and bleached by a co-existing free silver or the like during a long-term preservation.

In addition to the above disclosures, there are U.S. Pat. Nos. 3,180,732, 3,985,565, and 4,022,617; and Research Disclosure No. 12533 each disclosing the heat-developable color photo-sensitive materials utilizing a leuco dyes to produce a color image. In this process, however, there is a problem that the photo-sensitive materials are gradually colored during the preservation, 20 because it is difficult to incorporate the leuco dyes stably into the photo-sensitive materials.

In addition, Japanese Patent O.P.I. Publication No. 179840/1982 discloses a heat-developable color photo-sensitive material in which a color image pattern is formed by making use of a reducible dye-providing material capable of releasing both a dye-releasing assistant and a diffusible dye. In this method, however, it is inevitable to use the dye-releasing assistant, and this dye-releasing assistant is the so-called base or a basic precursor. There are the problems in the technique using such a base or a basic precursor, namely, fog is increased and a maximum density is lowered due to the existence of the base in the case of a heat-developable photo-sensitive material using an organic silver salt oxidizing agent.

Further, Japanese Patent O.P.I. Publication Nos. 186744/1982, 123533/1983 and 149046/1983 disclose the heat-developable color photo-sensitive materials in which a color transfer image pattern is obtained by releasing or producing a diffusible dye through a heat-development process. However, the exemplified compounds of the dye-providing materials disclosed therein have such a defect that it is hard to say that the migration of the compounds between the layers is completely prohibited during the multiple coating or heat-developing process, so that a color turbidity is apt to cause.

As disclosed in Japanese Patent O.P.I. Publication No. 149047/1983, there are the methods with the purpose of compensating the above-mentioned defect, in which a polymer is used to serve as a dye-providing material. Even the exemplified compounds described therein have the defects that, though the migration of dye-providing material is successfully prohibited, the efficiency of producing diffusible dye is substantially low and a maximum density (D<sub>max</sub>) of a transfer image pattern or the fog (D<sub>min</sub>) thereof is serious.

## SUMMARY OF THE INVENTION

It is an object of the invention to solve the problems inhering in the above-mentioned dye-providing materials, that it to say, it is an object of the invention to provide a heat-developable color photo-sensitive material containing a novel dye-providing material.

Another object of the invention is to provide a heat-developable color photo-sensitive material capable of obtaining a color image pattern which is less in color 5 turbidity and sharp in reproducibility.

A further object of the invention is to provide a dye-providing polymer which is excellent in efficiency of producing a diffusible dye.

A still further object of the invention is to provide a 10 yellow-dye-providing polymer capable of obtaining a transfer image pattern which is high in density and less in foginess.

The present inventors have devoted themselves in their studies with the purpose of achieving the above-mentioned objects, and consequently, the inventors have found that the objects of the invention can be achieved by a heat-developable color photo-sensitive material comprising a support bearing thereon a photographic component layer containing at least a photo-sensitive silver halide, a reducing agent, a binder and a 15 dye-providing material, among which at least one of the dye-providing material is a polymer having a repetition unit being derived from a monomer represented by the Formula [I] below;



Wherein,  $\text{R}_1$  represents an alkyl group;  $\text{R}_2$  represents an alkyl or an aryl group;  $\text{R}_3$  represents a divalent hydrocarbon;  $\text{R}_4$  represents an alkyl group or a hydrogen atom;  $\text{J}$  represents a divalent bonded group;  $1$  is an integer of 0 or 1; and  $m$  is an integer of 0 or 1.

## DETAILED DESCRIPTION OF THE INVENTION

In the abovegiven Formula [I],  $\text{R}_1$  represents an alkyl group which is allowed to have a substituent. The alkyl group represented by  $\text{R}_1$  is, preferably, a straight- or branched-chain alkyl group having not more than six carbon atoms which includes, for example, a methyl group, an ethyl group, an iso-propyl group, a tert-butyl group, an n-hexyl group. An alkyl group represented by  $\text{R}_1$  is, most preferably, a tert-butyl group.

In the abovegiven Formula [I],  $\text{R}_2$  represents an alkyl group or an aryl group, and these alkyl and aryl groups are allowed to have the respective substituents. The alkyl group represented by  $\text{R}_2$  includes a methyl group, an ethyl group, a benzyl group or the like. The aryl group represented by  $\text{R}_2$  includes a phenyl group, a naphthyl group or the like. Preferably,  $\text{R}_2$  is a phenyl group which is allowed to have a substituent.

In the abovegiven Formula [I],  $\text{R}_3$  represents a divalent hydrocarbon group which is allowed to have a substituent. The divalent hydrocarbon group includes, for example, an alkylene, arylene, aralkylene, alkylenearylene or arylenealkylene group, and the alkylene group includes, for example, methylene, ethylene, prop-

ylene group and the like; the arylene group includes, for example, phenylene group and the like; the aralkylene group includes, for example, phenylmethylene group and the like; the alkylenearylene group includes, for example, methylenephenoxy group and the like; the arylenealkylene group includes, for example, phenylenemethylene group and the like.

In the abovegiven Formula [I],  $\text{R}_4$  represents an alkyl group or a hydrogen atom, and the alkyl group represented by  $\text{R}_4$  is allowed to have a substituent. The alkyl group represented by  $\text{R}_4$  includes, preferably, an alkyl group having not more than 4 carbon atoms such as methyl, ethyl and n-butyl group.

In the abovegiven Formula [I],  $\text{J}$  represents a divalent bonded group, and the divalent bonded group represented by  $\text{J}$  includes, preferably,  $-\text{NHCO}$  or  $-\text{OCO}-$ .

As for substituents for the alkyl group represented by  $\text{R}_1$ , the alkyl or aryl group represented by  $\text{R}_2$ , the divalent hydrocarbon group represented by  $\text{R}_3$  and the alkyl group represented by  $\text{R}_4$  include, for example, a halogen atom such as fluorine, chlorine and bromine atom; a straight- or branched-chain alkyl group such as methyl, ethyl and t-butyl group; an aryl group such as phenyl group; an alkoxy group such as methoxy and ethoxy group; an acylamino group such as acetamide and benzamide group; an aryloxy group such as phenoxy group; an alkoxy carbonyl group such as methoxycarbonyl group; a nitro group; a hydroxyl group; and the like. These substituents are allowed to be two or more, and in the case of two or more of them, they are allowed to be the same or different from each other.

In the abovegiven Formula [I],  $1$  and  $m$  each are an integer of 0 or 1 respectively.

The polymers having a repetition unit being derived from monomer represented by the abovegiven Formula [I] (hereinafter referred to as dye-providing polymer of the invention) will form a diffusible dye through a coupling reaction with the oxidation product of the reducing agent. It is preferable for improving the diffusibility of the dye to be produced that  $\text{R}_1$  and  $\text{R}_2$  are so selected as to make the molecular weight of the coupler residual 55 group



not more than 700, and more preferably not more than 60 500.

Typical examples of the monomer compounds represented by the abovegiven Formula [I] of the invention are given below, and it is, however, to be understood that the invention shall not be limited thereto.



Y-1 5



Y-2



Y-3 40



Y-4 55



Y-5



Y-6



Y-7



Y-8



Y-9

-continued



-continued

Y-14

Y-10

5



10

15

Y-11 20

25

30

Y-12

40

45

Y-13



Y-15

Y-16

50 The polymers each having a repetition unit, which are derived from the monomeric compounds of the invention represented by the Formula [I], may be the so-called homopolymers each having a repetition unit, which comprise only one kind of the monomers represented by the Formula [I], or they may be the copolymers each comprising a combination of not less than two kinds of the monomers having the Formula [I], or they may further be copolymers each comprising one or more kinds of other comonomers each having copolymerizable ethylene unsaturated group.

55 As for the comonomers each having the above-mentioned ethylene unsaturated group, which are capable of forming a copolymer with the monomers of the invention having the Formula [I], there may be an ester acrylate, an ester methacrylate, a vinyl ester, an olefin, a styrene, an ester crotonate, a diester itaconate, a diester maleate, a diester fumarate, an acrylamide, an allyl compound, a vinyl ether, a vinyl ketone, a heterocyclic

vinyl compound, a glycidyl ester, an unsaturated nitrile, a polyfunctional monomer, a variety of unsaturated acids and the like.

These comonomers are more concretely exemplified as follows; the acrylic acid esters include, for example, methyl acrylate, ethyl acrylate, n-propyl acrylate, iso-propyl acrylate, n-butyl acrylate, isobutyl acrylate, sec-butyl acrylate, tert-butyl acrylate, amyl acrylate, hexyl acrylate, 2-ethyl hexyl acrylate, octyl acrylate, tert-octyl acrylate, 2-chloroethyl acrylate, 2-bromoethyl acrylate, 4-chlorobutyl acrylate, cyanoethyl acrylate, 2-acetoxyethyl acrylate, dimethylaminoethyl acrylate, benzyl acrylate, methoxybenzyl acrylate, 2-chlorocyclohexyl acrylate, cyclohexyl acrylate, furfryl acrylate, tetrahydrofurfuryl acrylate, phenyl acrylate, 5-15 hydroxypentyl acrylate, 2,2-dimethyl-3-hydroxypropyl acrylate, 2-methoxyethyl acrylate, 3-methoxybutyl acrylate, 2-ethoxyethyl acrylate, 2-iso-propoxy acrylate, 2-butoxyethyl acrylate, 2-(2-methoxyethoxy)ethyl acrylate, 2-(2-butoxyethoxy)ethyl acrylate,  $\omega$ -methoxypolyethyleneglycol acrylate, (added mol number n=9), 1-bromo-2-methoxyethyl acrylate, and 1,1-dichloro-2-ethoxyethyl acrylate.

The methacrylic acid esters include, for example, methyl methacrylate, ethyl methacrylate, n-propyl 25 methacrylate, isopropyl methacrylate, n-butyl methacrylate, isobutyl methacrylate, sec-butyl methacrylate, tert-butyl methacrylate, amyl methacrylate, hexyl methacrylate, cyclohexyl methacrylate, benzyl methacrylate, chlorobenzyl methacrylate, octyl methacrylate, sulfopropyl methacrylate, N-ethyl-N-phenylaminoethyl methacrylate, 2-(3-phenylpropoxy)ethyl methacrylate, dimethylaminophenoxyethyl methacrylate, furfuryl methacrylate, tetrahydrofurfuryl methacrylate, phenyl methacrylate, cresyl methacrylate, naphthyl methacrylate, 2-hydroxyethyl methacrylate, 4-hydroxybutyl methacrylate, triethyleneglycol monomethacrylate, dipropylene glycol monomethacrylate, 2-methoxyethyl methacrylate, 3-methoxybutyl methacrylate, 2-acetoxyethyl methacrylate, 2-acetoacetoxyethyl methacrylate, 2-ethoxyethyl methacrylate, 2-isopropoxyethyl methacrylate, 2-butoxyethyl methacrylate, 2-(2-methoxyethoxy)ethyl methacrylate, 2-(2-ethoxyethoxy)ethyl methacrylate, 2-(2-butoxyethoxy)ethyl methacrylate,  $\omega$ -methoxypolyethyleneglycol 30 35 40 methacrylate (added mol number n=6), allyl methacrylate and methacrylic acid dimethylaminoethyl methyl chloride salt.

The vinyl esters include, for example, vinyl acetate, vinyl propionate, vinyl butyrate, vinyl isobutyrate, vinyl 50 caproate, vinyl chloroacetate, vinyl methoxyacetate, vinyl phenylacetate, vinyl benzoate and vinyl salicylate.

The olefins include, for example, dicyclopentadiene, ethylene, propylene, 1-butene, 1-pentene, vinyl chloride, vinylidene chloride, isoprene, chloroprene, butadiene and 2,3-dimethylbutadiene.

The styrenes include, for example, styrene, methylstyrene, dimethylstyrene, trimethylstyrene, ethylstyrene, isopropylstyrene, chloromethylstyrene, methoxystyrene, acetoxy styrene, chlorostyrene, dichlorostyrene, bromostyrene and methyl vinylbenzoate.

The crotonic acid esters include, for example, butyl crotonate, hexyl crotonate and the like.

The itaconic acid diesters include, for example, dimethyl itaconate, diethyl itaconate, dibutyl itaconate and the like.

The maleic acid diesters include, for example, diethyl maleate, dimethyl maleate, dibutyl maleate and the like.

The fumaric acid diesters include, for example, diethyl fumarate, dimethyl fumarate, dibutyl fumarate and the like.

The examples of the other comonomers may be given as follows.

An acrylamide such as acrylamide, methylacrylamide, ethylacrylamide, propylacrylamido, butylacrylamide, tert-butylacrylamide, cyclohexylacrylamide, benzylacrylamide, hydroxymethylacrylamide, methoxyethylacrylamide, dimethylaminoethylacrylamide, phenylacrylamide, dimethylacrylamide, diethylacrylamide,  $\beta$ -cyanoethylacrylamide and N-(2-acetoacetoxyethyl)acrylamide;

A methacrylamide such as methacrylamide, methylmethacrylamide, ethylmethacrylamide, propylmethacrylamide, butylmethacrylamide, tert-butylmethacrylamide, cyclohexylmethacrylamide, benzylmethacrylamide, hydroxymethylmethacrylamide, methoxyethylmethacrylamide, dimethylaminoethylmethacrylamide, phenyl methacrylamide diethylmethacrylamide, dimethylmethacrylamide,  $\beta$ -cyanoethylmethacrylamide and N-(2-acetoacetoxyethyl)methacrylamide.

An allyl compound, such as allyl acetate, allyl caproate, allyl laurate and allyl benzoate;

A vinylether, such as methylvinylether, butylvinylether, hexylvinylether, methoxyethylvinylether and dimethylaminoethylvinylether;

A vinylketone, such as methylvinylketone, phenylvinylketone and methoxyethylvinylketone;

A vinylheterocyclic compound, such as vinylpyridine, N-vinylimidazole, N-vinyloxazolidone, N-vinyltriazole and N-vinylpyrrolidone;

A glycidyl ester, such as glycidyl acrylate and glycidyl methacrylate;

An unsaturated nitrile such as acrylonitrile and methacrylonitrile;

A multi functional monomer, such as divinylbenzene, methylenebisacrylamide and ethyleneglycol dimethacrylate.

Further, the monomer are given as acrylic acid, methacrylic acid, itaconic acid, maleic acid and a mono-alkyl itaconate such as monomethyl itaconate, monoethyl itaconate and monobutyl itaconate; a monoalkyl maleate such as monomethyl maleate, monoethyl maleate and monobutyl maleate; citraconic acid, stylenesulfonic acid, vinylbenzylsulfonic acid, vinylsulfonic acid, an acryloyloxyalkylsulfonic acid such as acryloyloxyalkylsulfonic acid, acryloyloxyethylsulfonic acid, acryloyloxypropylsulfonic acid; a methacryloxyalkylsulfonic acid such as methacryloxyloxyalkylsulfonic acid, methacryloyloxyethylsulfonic acid and methacryloylpropylsulfonic acid; an acrylamidoalkylsulfonic acid such as 2-acrylamide-2-methylethanesulfonic acid, 2-acrylamide-2-methylpropanesulfonic acid and 2-acrylamide-2-methylbutanesulfonic acid; a methacrylamidoalkylsulfonic acid such as 2-methacrylamide-2-methylethanesulfonic acid, 2-methacrylamide-2-methylpropanesulfonic acid, 2-methacrylamide-b 2-methylbutanesulfonic acid, an acryloyloxyethylphosphate and 3-acryloyloxypropyl-2-phosphate; a methacryloyloxyalkylphosphate such as methacryloyloxyethylphosphate and 3-methacryloyloxypropyl-2-phosphate; and a 3-allyoxy-2-hydroxypropanesulfonic acid having two hydrophilic groups, such as 3-alloxy-2-sodium-hydroxypropanesulfonate. These acids may also be such an alkaline metal as Na, K and the like, or an ammonium ion salt. As for the other comonomers, such a bridged

monomer as described in U.S. Pat. Nos. 3,459,790, 3,438,708, 3,554,987, 4,215,195 and 4,247,673, and Japanese Patent O.P.I. Publication No. 205735/1982 may be used. To be more concrete, they include, for example, N-(2-acetoacetoxyethyl)acrylamide, N-[2-(2-acetoacetoxyethoxyethyl)acrylamide, and the like.

In the case of forming a copolymer by making use of a monomer of the invention having the Formula [I] and the aforementioned comonomer, a preferable case thereof is that the contents of the repetition unit comprising a monomer having the Formula [I] are from 10 wt% to 90 wt% of the whole polymer, and more preferable case is that the contents thereof are 30 wt% to 70 wt% of the whole polymer.

In general, a polymer coupler is prepared in an emulsion-polymerization process or in a solution-polymerization process. The same processes may be applied to the dye-providing polymers of the invention having the repetition unit derived from the monomers of the invention having the Formula [I]. As for the emulsion-polymerization processes, those described in U.S. Pat. Nos. 4,080,211 and 3,370,952 may be applied, and as for the processes in which hydrophilic polymers are dispersed to serve as the latex into an aqueous solution of gelatin, those described in U.S. Pat. No. 3,451,820 may be applied.

These processes may also be applied to form a homopolymer or copolymer. In the latter case, the comonomers thereof may be liquid comonomers which may serve, in a normal state, as a solvent for a stationary monomer, when emulsification-polymerizing.

As for the emulsifying agents to be applicable to the emulsification-polymerization process, these include a surface active agent, a macromolecular protective colloid, and a copolymeric emulsifying agent. As for the surface active agents, there include, for example, an anionic active agent, a nonionic active agent, a cationic active agent, and an amphoteric active agent.

As for the anionic active agent, there are given as the examples, a soap, sodium dodecylbenzene sulfonate, sodium laurylsulfate, sodium dioctylsulfosuccinate, and a sulfuric acid salt of a nonionic active agent.

As for the nonionic active agents, there include, for example, a polyoxyethylene nonylphenyl ether, a polyoxyethylene stearic acid ester, a polyoxyethylene sorbitan monolaurylic acid ester, a polyoxyethylene-polyoxypolypropylene block copolymer, and the like. As for the cationic active agents, there include, for example, an alkylpyridium salt, tertiary amine and the like.

As for the amphoteric active agents there include, for example, a dimethyl alkyl betaine, an alkyl glycine and the like. As for the macromolecular protective colloids, there include, for example, a polyvinyl alcohol, hydroxyethyl cellulose and the like. They may be used independently to serve as an emulsifying agent and may also be used in combination with the other surface active agents. The various kinds and functions of these active agents are described in 'Belgische Chemische Industrie, 28, 16-20 (1963)'.

How to disperse a lipophilic polymer synthesized in a solution polymerization process into an aqueous gelatin solution so that the polymer may be dispersed therein in the form of a latex, the lipophilic polymer is dissolved in an organic solvent first and the solution thereof is then dispersed latexwise in an aqueous gelatin solution, with the aid of a dispersing agent, by means of a supersonic colloid-mill or the like. The processes of dispersing a lipophilic polymer in the form of a latex into an aqueous

gelatin solution are described in U.S. Pat. No. 3,451,820. As for the organic solvents for dissolving the lipophilic polymers, there include, for example, esters such as methyl acetate, ethyl acetate, propyl acetate, and the like, and an alcohol, a ketone, a halogenated hydrocarbon, an ether, and the like. These organic solvents may be used independently or in combination with two or more kinds of them.

In the case of preparing a dye-providing polymer relating to this invention, it is desired that the solvents to be used in a polymerization process are a monomer and a well-qualified solvent for dye-providing polymers to be produced, and are relatively low in reactivity with a polymerization starting agent. To be more concrete, there include, for example, water, toluene, an alcohol (e.g., methanol, ethanol, iso-propanol, tert-butanol and the like), acetone, methyl ethyl ketone, tetrahydrofuran, dioxane, ethyl acetate, dimethyl formamide, dimethyl sulfoxide, acetonitrile, methylene chloride, and the like; and these solvents may be used independently or in a mixture of two or more kinds thereof.

The temperatures for a polymerization process are normally within the range of from 30° C. to 120° C., though it is necessary to take the kinds of the polymerization starting agents and the solvents into consideration.

As for the polymerization starting agents to be used in the emulsification-polymerization process or the solution-polymerization process for preparing a dye-providing polymer of this invention, there include the following ones:

As for a water-soluble polymerization starting agent, there include, for example, a persulfate such as potassium persulfate, ammonium persulfate, sodium persulfate and the like; a water-soluble azo compound such as 4,4'-azobis-4-sodium cyanovaleate, 2,2'-azobis(2-amidinopropane) chloride and the like; and hydrogen peroxide.

As for the lipophilic polymerization starting agents to be used in the solution-polymerization process, there include, for example, an azo compound such as azobisisobutyronitrile, 2,2'-azobis-(2,4-dimethylvaleronitrile), 2,2'-azobis-(4-methoxy-2,4-dimethylvaleronitrile), 1,1'-azobis(cyclohexanon-1-carbonitrile), 2,2'-azobisisocyanobutyric acid, 2,2'-dimethylazobisisobutyrate, 1,1'-azobis(cyclohexanone-1-carbonitrile), 4,4'-azobis-4-cyanovaleeric acid; a peroxide compound such as benzoyl peroxide, lauryl peroxide, chlorobenzyl peroxide, diisopropyl peroxycarbonate and di-t-butyl peroxide. The preferable ones among the above are benzoyl peroxide, chlorobenzyl peroxide, lauryl peroxide and the like.

These polymerization starting agents may be contained in the range of from 0.01 wt% to 10 wt% and more preferably from 0.1 wt% to 5 wt% to the aggregate quantity of monomers in the emulsification-polymerization process or in the solution-polymerization process.

Besides the above-mentioned processes, the other processes such as a suspension-polymerization process, a block-polymerization and the like may also be applied. In other words, in this invention, there contains every one of the dye-providing homopolymer of the monomers of the invention having the Formula [I], a copolymer comprising two or more of the monomers in combination, or a copolymer comprising the monomers and at least one kind of the other polymerizable comonomers

as the copolymeric components. The invention shall not be limited to the synthesizing processes.

The following dye-providing polymers of the invention are given as the typical examples. It is, however, to be understood that the invention shall not be limited thereto.

Exemplified dye-providing polymer

PY-1

exemplified monomer (1)-butylacrylate copolymer (polymerization ratio 1:1)

PY-2

exemplified monomer (1)-butylacrylate copolymer (polymerization ratio 3:2)

PY-3

exemplified monomer (1)-butylacrylate copolymer (polymerization ratio 7:3)

PY-4

exemplified monomer (1)-methylmethacrylate copolymer (polymerization ratio 6:4)

PY-5

exemplified monomer (2)-butylacrylate copolymer (polymerization ratio 7:3)

PY-6

exemplified monomer (3)-butylacrylate copolymer (polymerization ratio 2:3)

PY-7

exemplified monomer (4)-butylacrylate copolymer (polymerization ratio 3:7)

PY-8

exemplified monomer (5)-2-ethylhexylacrylate copolymer (polymerization ratio 3:2)

PY-9

exemplified monomer (1)-p-sulfostyrene copolymer (polymerization ratio 2:3)

PY-10

exemplified monomer (1)-2-hydroxyethylacrylate copolymer (polymerization ratio 1:1)

PY-11

exemplified monomer (1)-vinyl pyrrolidone copolymer (polymerization ratio 7:3)

PY-12

exemplified monomer (11)-butylacrylate copolymer (polymerization ratio 3:2)

PY-13

exemplified monomer (11)-octylacrylate copolymer (polymerization ratio 3:2)

PY-14

exemplified monomer (11)-acrylic acid-vinyl pyrrolidone copolymer (polymerization ratio 2:1:2)

(Provided that polymerization ratio means weight ratio.)

Synthesis examples of the above-mentioned dye-providing polymers of the invention will be given below:

SYNTHESIS EXAMPLE 1

Synthesis of Exemplified Dye-providing Polymer (PY-1)

A solution was prepared by adding 10 g of the exemplified monomer (Y-5) and 10 g of butyl acrylate into 100 ml of dioxane and the resulting solution was heated up to 80°~82° C. under nitrogen air-flow. With keeping the temperature, 300 mg of 2,2-azobisisobutyronitrile

were added and a reaction was made for four hours. After completing the reaction, the resulting reactant liquid was poured into one liter of water and the precipitates thereof were filtrated and dried. Thus, the objective polymer (PY-1) was obtained.

It is preferred that the molecular weight of a dye-providing polymer of the invention is within the range of from 1,500 to 100,000 in term of weight-average molecular weight (Mw).

- 10 Any dye-providing polymer of the invention may be used independently or in combination. The amount thereof to be used is not limited but may be depended upon the kinds of the polymers, whether they are to be used independently or in combination with two or more of them or whether the photographic component layer of the photo-sensitive material of the invention is single-layered or multi-layered with two or more layers. For example, an amount to be used is from 0.005 g to 10 g and preferably from 0.1 g to 5.0 g per square-meter of a support.

Any arbitrary process may be applied to contain a dye-providing polymer of the invention in the photographic component layers of a heat-developable color photo-sensitive material. For example, the polymers of the invention may be contained in the component layer in such a manner that the polymers are dissolved in a low-boiling solvent such as methanol, ethanol, ethyl acetate or the like, or a high-boiling solvent such as dibutyl phthalate, dioctyl phthalate, tricresyl phosphate, or the like and the resulted solution is then dispersed by ultrasonic waves; that the polymers are dissolved in an aqueous alkali solution such as an aqueous solution of 10% sodium hydroxide or the like and the

- 25 resulted solution is neutralized by a mineral acid such as chloric acid, nitric acid or the like; or that the polymers are dispersed together with an aqueous solution of a suitable polymer such as gelatin, polyvinyl butyral, polyvinyl pyrrolidone, or the like, by making use of a ball-mill.
- 30 A heat-developable color photo-sensitive material of the invention contains a photo-sensitive silver halide as well as the above-mentioned dye-providing polymer of the invention.

- 35 40 45 The photo-sensitive silver halide to be used in the invention include, for example, silver chloride, silver bromide, silver iodide, silver chlorobromide, silver chloroiodide, silver iodobromide, silver chloroiodobromide, and the like. These photo-sensitive silver halide can be prepared in such an arbitrary process in the photographic technical field as a single-jet process, a double-jet process and the like. In the invention, the desired results are obtained with the use of photo-sensitive silver halide emulsions containing a photo-sensitive silver halide prepared in accordance with an ordinary preparation process of a silver halide gelatin emulsion.

- 50 55 60 Such photo-sensitive silver halide emulsions may also be chemically sensitized in an arbitrary process used in the photographic technical field. As for such sensitizing processes, there are various processes including, for example, a gold sensitization, a sulphur sensitization, a gold-sulphur sensitization, a reduction sensitization, and the like.

The silver halide of the above-mentioned photo-sensitive emulsions may be either coarse grain or fine grain. The preferred grain sizes are from about 0.001 μm to about 1.5 μm in diameter and more preferably from about 0.01 μm to about 0.5 μm.

The photo-sensitive silver halide emulsions prepared as mentioned above can be most preferably applied to a heat-developable photo-sensitive layer that is a component layer of the photo-sensitive materials of this invention.

As for a process of preparing the other photo-sensitive silver halide, it is also possible, in this invention, to form a photo-sensitive silver halide in a portion of an organic silver salt by making a photo-sensitive silver salt forming component co-exist with an organic silver salt which will be described later. As for the photo-sensitive silver salt forming components to be used in this preparing process, an inorganic halide may be given as the example thereof, including, for example; a halide represented by  $MX_n$  in which  $M$  represents hydrogen,  $NH_4$  group or a metal atom,  $X$  represents  $Cl$ ,  $Br$  or  $I$  and  $n$  is 1 when the  $M$  is hydrogen or  $NH_4$  group, and when  $M$  is a metal atom,  $n$  is the valence thereof, and the metal atoms include those of lithium, sodium, potassium, rubidium, cecium, copper, gold, beryllium, magnesium, calcium, strontium, barium, zinc, cadmium, mercury, aluminum, indium, lanthanum, ruthenium, thalium, germanium, tin, lead, antimony, bismuth, chromium, molybdenum, wolfram, manganese, rhenium, iron, cobalt, nickel, rhodium, paradium, osmium, iridium, platinum, cerium; a halide-containing metal complex, such as  $K_2PtCl_6$ ,  $K_2PtBr_6$ ,  $HAuCl_4$ ,  $(NH_4)_2IrCl_6$ ,  $(NH_4)_3IrCl_6$ ,  $(NH_4)_2RuCl_6$ ,  $(NH_4)_3RuCl_6$ ,  $(NH_4)_3RhCl_6$ ,  $(NH_4)_3RhBr_6$ ; an onium halide e.g., a quaternary ammonium halide such as tetramethylammonium bromide, trimethylphenylammonium bromide, cetylthyldimethylammonium bromide, 3-methylthiazolium bromide and trimethylbenzylammonium bromide; a quaternary phosphonium halide such as tetraethylphosphonium bromide; a tertiary sulfonium halide such as benzylethylmethylsulfonium bromide and 1-ethylthiazolium bromide; a halogenated hydrocarbon, such as iodoform, bromeform, carbontetrachloride and 2-bromo-2-methylpropane; an N-halogen compound such as N-chlorosuccinimide, N-bromosuccinimide, N-bromophthalimide, N-bromoacetamide, N-iodosuccinimide, N-bromophthaladinone, N-chlorophthaladinone, N-bromoacetanilide, N,N-dibromobenzensulfonamide, N-bromo-N-methylbenzensulphonamide and 1,3-dibromo-4,4-dimethylhydantoin; and the other halogen containing compounds such as triphenylmethyl chloride, triphenylmethyl bromide, 2-bromobutyric acid, and 2-bromoethanol.

These photo-sensitive silver halide and the photo-sensitive silver salt forming components may be used in combination in various processes. A preferable amount used thereof is from 0.001 g to 50 g, and a more preferable amount is from 0.1 g to 10 g per square meter of a layer.

The heat-developable color photo-sensitive materials of the invention may comprise each of blue-light-sensitive, green-light-sensitive and red-light-sensitive layers, namely, a multiple-layer comprising a heat-developable blue-light-sensitive layer, a heat-developable green-light-sensitive layer and a red-light-sensitive layer, and the same light-sensitive layer thereof may be divided into two or more layers such as a combination of a high sensitive layer and a low sensitive layer.

Each of the blue-light sensitive silver halide emulsion, green-light sensitive silver halide emulsion and red-light-sensitive silver halide emulsion to be used in the above-mentioned case may be prepared by adding vari-

ous kinds of spectral sensitization dyes to the silver halide emulsions.

The spectral sensitization dyes which may typically be used in this invention include, for example, cyanine, merocyanine, a trinuclear or tetrnuclear complex cyanine, holopolar cyanine, styryl, hemicyanine, oxonole and the like. Among the cyanine dyes, those each having a basic nucleus such as thiazoline, oxazoline, pyrrole, pyridine, oxazole, thiazole, selenazole, and imidazole are preferred to use. Such a nucleus may have an enamine group capable of producing an alkyl group, alkylene group, hydroxyalkyl group, sulfoalkyl group, carboxyalkyl group, aminoalkyl group, or a condensed carbocyclic or heterocyclic color ring. Also, it may be in the symmetric or unsymmetric form, and the methine chain or the polymethine chain thereof may have an alkyl group, a phenyl group, an enamine group and a heterocyclic substituent.

Besides the above-mentioned basic nuclei, the merocyanine dyes may also have, for example, such an acid nucleus as a thiohydantoin nucleus, a rhodanine nucleus, an oxazolyl acid nucleus, a thiazolinethione nucleus, a malononitrile nucleus, and a pyrazolone nucleus. These acid nuclei may also be substituted by either of an alkyl, alkylene, phenyl, carboxyalkyl, sulfoalkyl, hydroxyalkyl, alkoxyalkyl or alkylamine group, or a heterocyclic ring nucleus. If required, these dyes may further be used in combination. It is still further possible to jointly use such a supersensitive additive incapable of absorbing any visible rays of light as an ascorbic acid derivative, an azaindene cadmium salt, an organic sulfonic acid and the like including, for example, those described in U.S. Pat. Nos. 2,933,390, and 2,937,089.

The amount of these dyes to be added is from  $1 \times 10^{-4}$  mole to 1 mole per mol of a silver halide or a silver halide forming component, and more preferably, from  $1 \times 10^{-4}$  mole to  $1 \times 10^{-1}$  mole.

In the heat-developable color photo-sensitive materials of the invention, various kinds of organic silver salts may be used if required for increasing the sensitivity and improving the developability of the materials.

As for the organic silver salts to be used to the heat-developable color photo-sensitive materials of the invention, there may be given as the examples thereof the following: an aliphatic carboxylic acid silver salt such as silver laurate, silver myristate, silver palmitate, silver stearate, silver arachidonate, silver behenate, silver  $\beta$ -(1-phenyltetrazolethio) acetate and the like, an aromatic silver carboxylate such as silver benzoate, silver phthalate and the like, as described in Japanese Patent Examined Publication Nos. 4921/1968, 26582/1969, 18416/1970, 12700/1970, and 22185/1970, Japanese Patent O.P.I. Publication No. 52626/1974, 31728/1977, 137321/1977, 141222/1977, 36224/1978 and 37610/1978, and U.S. Pat. Nos. 3,330,633, 3,794,496, 4,105,451, 4,123,274 and 4,168,980, and the like; and silver salts of an imino group, for example, those of benzotriazole, 5-nitrobenzotriazole, 5-chlorobenzotriazole, 5-methoxybenzotriazole, 4-sulfonylbenzotriazole, 4-hydroxybenzotriazole, 5-aminobenzotriazole, 5-carboxybenzotriazole, imidazole, benzimidazole, 6-nitrobenzimidazole, pyrazole, urazol, 1,2,4-triazole, 1H-tetrazole, 3-amino-5-benzylthio-1,2,4-triazole, saccharin, phthalazinone, phthalimide, and besides, those of 2-mercaptopbenzoxazole, mercaptoxydiazole, 2-mercaptopbenzothiazole, 2-mercaptopbenzimidazole, 3-mercaptop-4-phenyl-1,2,4-triazole, 4-hydroxy-6-methyl-

1,3,3a,7-tetrazaindene, and 5-methyl-7-hydroxy-1,2,3,4,6-pentazaindene, as described in Japanese Patent Examined Publication Nos. 26582/1969, 12700/1970, 18416/1970 and 22185/1970, Japanese Patent O.P.I. Publication Nos. 31728/1977, 137321/1977, 118638/1983 and 118639/1983. Among the above-mentioned organic silver salts, silver salts of an imino group are preferred to use, especially silver salts of a benzotriazole derivative are preferred, and further, silver salts of a sulfonylbenzotriazole derivative are more preferred to use.

The organic silver salts to be used in the invention may be used independently or in combination with two or more kinds thereof. They may also be used in such a manner that they are isolated and are then dispersed in a binder by a suitable means, or in such a manner that a silver salt is prepared in a suitable binder and the resulted silver salt is used as it is without applying any isolation.

The amount of the above-mentioned organic silver salts to be used is preferably from 0.01 mol to 500 mol and more preferably from 0.1 mol to 100 mol, per mol of a photo-sensitive silver halide.

The reducing agents to be used in the heat-developable color photo-sensitive materials of the invention are those which are popularly used in the field of heat-developable color photo-sensitive materials. There may be given as the examples thereof the developing agents of p-phenylenediamine type, p-aminophenol type, phosphoramidophenol type, sulfonamidophenol type or hydrazone type color developing agent, described in, for example, U.S. Pat. Nos. 3,531,286, 3,761,270, and 3,764,328, Research Disclosure Nos. 12146, 15108 and 15127, and Japanese Patent O.P.I. Publication No. 27132/1981. There may also be used advantageously the color developing agent precursors and the like which are described in U.S. Pat. Nos. 3,342,599, and 3,719,492, and Japanese Patent O.P.I. Publication Nos. 135,628/1978 and 79035/1979.

The particularly preferable reducing agents may be given those represented by the following formula [II] appeared in Japanese Patent O.P.I. Publication No. 146133/1981:



Wherein, R<sub>5</sub> and R<sub>6</sub> each represent hydrogen or an alkyl group which is allowed to have a substituent and has one to 30 carbon atoms and preferably one to four carbon atoms, and the R<sub>5</sub> and R<sub>6</sub> may close a ring so as to form a heterocyclic ring; R<sub>7</sub>, R<sub>8</sub>, R<sub>9</sub> and R<sub>10</sub> each represent hydrogen, a halogen, a hydroxy group, an amino group, an alkoxy group, an acylamide group, a sulfonamide group, an alkylsulfonamide group, or an alkyl group which is allowed to have a substituent and has one to 30 carbon atoms, and preferably, one to four carbon atoms, and the R<sub>7</sub> and R<sub>5</sub>, and the R<sub>9</sub> and R<sub>6</sub> each may close a ring so as to form a heterocyclic ring, respectively; and M represents an alkaline metal atom or a compound containing an ammonium group, a nitrogen-containing organic base or a quaternary nitrogen atom.

The nitrogen-containing organic base in the Formula [II] is an organic compound containing a nitrogen atom which is capable of producing an inorganic acid and a salt and displays a basicity. The particularly essential organic bases include, for example, an amine compound. Chain amine compounds include, for example, primary amine, secondary amine, and tertiary amine, and cyclic amine compounds include pyridine, quinoline, piperidine, imidazole and the like as the famous examples of the typical heterocyclic organic bases. Besides the above, such a compound as hydroxylamine, hydrazine, amidine and the like is also useful for a chain amine. As for the salts of nitrogen-containing organic bases, such an inorganic acid salt as a chloride, a sulfate, a nitrate or the like of the organic bases is preferably used.

On the other hand, as for the compounds each containing quaternary nitrogen in the formula above, there include, for example, a salt or hydroxide of a nitrogen compound having a quadrivalent covalent bond.

Next, some preferred examples of the reducing agents represented by Formula [II] above will be given below:



-continued



-continued

(R-19)



35 The reducing agents represented by Formula [II] may be synthesized in such a well-known process as described in, for example, Houben-Weyl, Methoden der Organischen Chemie, Band XI/2, pp. 645-703.

40 Besides the above, there may be used such a group of reducing agents as exemplified below;

45 A phenol (e.g., p-phenylphenol, p-methoxyphenol, 2,6-di-tert-butyl-p-cresol, N-methyl-p-aminophenol), a sulfonamidophenol (e.g., 4-benzensulfonamidophenol, 2-benzensulfonamidophenol, 2,6-dichloro-4-benzenesulfonamidophenol, 2,6-dibromo-4-(p-toluenesulfonamide)phenol), and a polyhydroxybenzene (e.g., hydroquinone, tert-butylhydroquinone, 2,6-dimethylhydroquinone, chlorohydroquinone, carboxyhydroquinone, catechol, 3-carboxycatechol), a naphthol (e.g.,  $\alpha$ -naphthol,  $\beta$ -naphthol, 4-aminonaphthol, 4-methoxy- $\alpha$ -naphthol), a hydroxybinaphthyl and methylenebis-naphthol (e.g., 1,1'-dihydroxy-2,2'-binaphthyl, 6,6'-dibromo-2,2'-dihydroxy-1,1'-binaphthyl, 6,6'-dinitro-2,2'-dihydroxy-1,1'-binaphthyl, 4,4'-dimethoxy-1,1'-dihydroxy-2,2'-binaphthyl, bis(2-hydroxy-1-naphthyl)methane), a methylenebisphenol (e.g., 1,1-bis(2-hydroxy-3,5-dimethylphenyl)-3,5,5-trimethylhexane, 1,1-bis(2-hydroxy-3-tert-butyl-5-methylphenyl)methane, 1,1-bis(2-hydroxy-3,5-di-tert-butylphenyl)methane, 2,6-methylene-bis(2-hydroxy-3-tert-butyl-5-methylphenyl)-4-methylphenol,  $\alpha$ -phenyl- $\alpha$ -bis(2-hydroxy-3,5-dimethylphenyl)-2-methylpropane,  $\alpha$ -phenyl- $\alpha$ , $\alpha$ -bis(2-hydroxy-3-tert-butyl-5-methylphenyl)methane, 1,1-bis(2-hydroxy-3,5-dimethylphenyl)-2-methylpropane, 1,1,5,5-tetrakis(2-hydroxy-3,5-dimethylphenyl)-2,4-ethylpentane, 2,2-bis(4-hydroxy-3,5-dimethylphenyl)-propane, 2,2-bis(4-hydroxy-3-methyl-5-tert-butyl-

phenyl)propane, 2,2-bis(4-hydroxy-3,5-di-tert-butyl-phenyl)propane}, an ascorbic acid, a 3-pyrazolidone, a pyrazolone, a hydrazone, and a paraphenylenediamine.

These reducing agents may be used independently or in combination with two or more thereof. An amount of the reducing agents used depends upon the kinds of photo-sensitive silver halide, the kinds of organic acid silver salts and the kinds of the other additives, and is normally from 0.01 mole to 1500 mole per mole of a photo-sensitive silver halide, and more preferably, from 0.1 mole to 200 mole.

As for the binders to be used in the heat-developable color photo-sensitive materials of the invention, there may be used independently or in combination of two or more synthetic or natural high molecular substances such as polyvinyl butyral, polyvinyl acetate, ethyl cellulose, polymethyl methacrylate, cellulose acetate butylate, polyvinyl alcohol, polyvinyl pyrrolidone, gelatin and phthalic gelatin. In particular, it is preferable to use gelatin or the derivatives thereof in combination with such a hydrophilic polymer as polyvinyl pyrrolidone, polyvinyl alcohol or the like, and it is more preferable to use the under-mentioned binders described in Japanese Patent Application No. 104249/1983.

This binder contains gelatin and a vinyl pyrrolidone polymer. The vinyl pyrrolidone polymer may be a polyvinyl pyrrolidone which is a homopolymer of vinyl pyrrolidone or may be a copolymer, including a graft copolymer, of vinyl pyrrolidone and one or two of the other monomers capable of polymerizing with the vinyl pyrrolidone. These polymers may be used regardless of any polymerization degree thereof. The polyvinyl pyrrolidone may be a substituted polyvinyl pyrrolidone, and a preferred polyvinyl pyrrolidone has a molecular weight of from 1,000 to 400,000. As for the other monomers capable of copolymerizing with vinyl pyrrolidone, there are vinyl monomers including, for example, a (meth) acryl ester such as acrylic acid, methacrylic acid and the alkyl esters thereof, a vinyl alcohol, a vinyl imidazol, a (meth) acrylamide, a vinyl carbinol, a vinyl alkyl ether and the like. It is preferred that at least 20% by weight of the composition thereof (hereinafter a percentage by weight will be referred simply to as '%') is polyvinyl pyrrolidone. In the preferred examples of such polymers, their molecular weight each are from 5,000 to 400,000.

The gelatins may be treated in a liming or acidizing process, and they may also be an ossein gelatin, a pig-skin gelatin, a hide gelatin or a denatured gelatin in which the above-mentioned gelatin is esterified, or phenylcarbamoylated.

In the above-mentioned binders, a gelatin amount to the total binder amount is preferably from 10% to 90% and more preferably from 20% to 60%, and the amount of vinyl pyrrolidone thereto is preferably from 5% to 90% and more preferably from 10% to 80%.

The above-mentioned binders may contain other high molecular substances, and the preferred binders comprise, for example, gelatin and a mixture of polyvinyl pyrrolidone of from 1,000 to 400,000 in molecular weight and one or more than two of other high molecular substances, or they comprise gelatin and a mixture of a vinyl pyrrolidone copolymer of from 5,000 to 400,000 in molecular weight and one or more than two of other high molecular substances. As for the other high molecular substances to be used therein, there may be given as the examples, polyvinyl alcohol, polyacrylamide, polymethacrylamide, polyvinyl butyral, polyethylene

glycol, a polyethylene glycol ester, or a natural substance including, for example, a protein such as a cellulose derivative, and a polysaccharide such as starch and gum arabic. The contents thereof may be from 0 to 85% and preferably from 0 to 70%.

In addition, the above-mentioned vinyl pyrrolidone polymers may also be a cross-linked polymers, and if this is the cause, it is preferred to make them cross-link after they are coated on a support. This case include the case where a cross-linking reaction is progressed in nature.

The amount of the binders used therein is normally from 0.005 g to 50 g per square meter of a layer, and more preferably from 0.1 g to 10 g. The binders are to be used preferably in the amount from 0.1 g to 10 g per gram of a dye-providing material monomer unit, and more preferably in the amount of from 0.25 g to 4 g.

Supports used for the heat-developable color photo-sensitive materials of the invention include, for example, synthetic plastic films such as polyethylene film, cellulose acetate film, polyethylene terephthalate film and polyvinyl chloride, paper supports such as photographic base paper, printing paper, baryta paper and resin-coated paper, and supports in which a reflective layer is provided to the above-given synthetic plastic films.

In particular, the heat-developable color photo-sensitive materials of the invention are preferably added with a variety of thermal solvents. Any substances capable of accelerating a heat-development and/or a heat-transfer can serve as a thermal solvent of the invention. They are preferably a solid, semi-solid or liquid substance (preferably, at atmospheric pressure, boiling point is not less than 100° C. and more preferably not less than 150° C.) capable of being dissolved or fused in a binder when it is heated up, and those include, as the preferably ones, a urea derivative such as dimethylurea, diethylurea and phenylurea; an amide derivative such as acetamide, and benzamide; a polyhydric alcohol such as 1,5-pentanediol, 1,6-pentanediol, 1,2-cyclohexanediol, pentaerythritol, and trimethylethane; or a polyethylene glycol. More typical examples are given in Japanese Patent Application No. 104249/1983. These thermal solvents may be used independently or in combination.

To the heat-developable color photo-sensitive material of the invention, if necessary, various additives may be added other than each constituents described above. For example, development accelerators include alkali-releasing agents such as urea and guanidium trichloroacetate described in U.S. Pat. Nos. 3,220,840, 3,531,285, 4,012,260, 4,060,420, 4,088,496 and 4,207,392, Research Disclosure Nos. 15733, 15734 and 15776, Japanese Patent O.P.I. Publication Nos. 130745/1981 and 132332/1981; an inorganic acid described in Japanese Patent Examined Publication No. 12700/1970; non-aqueous polar solvent compounds having —CO—, —SO<sub>2</sub>— and —SO— group described in U.S. Pat. No. 3,667,959; Melformer described in U.S. Pat. No. 3,438,776; polyalkylene glycol described in U.S. Pat. No. 3,666,477 and Japanese Patent O.P.I. Publication No. 19525/1976. As for the color tone control agents, those compounds disclosed in Japanese Patent O.P.I. Publication Nos. 4928/1971, 6077/1971, 5019/1974, 5020/1974, 91215/1974, 107727/1974, 2524/1975, 67132/1975, 67641/1975, 114217/1975, 33722/1977, 99813/1977, 1020/1978, 55115/1978, 76020/1978, 125014/1978, 156523/1979, 156524/1979, 156525/1979, 156526/1979, 4060/1980, 4061/1980 and 32015/1980;

West German Pat. Nos. 2140406, 2147063 and 2220618; U.S. Pat. Nos. 3,080,254, 3,847,612, 3,782,941, 3,994,732, 4,123,282 and 4,201,582 may be used. Examples thereof are phthalazinone, phthalimide, pyrazolone, quinazolinone, N-hydroxynaphthalimide, benzoxazine, naphthoxazinedione, 2,3-dihydro-phthalazinedione, 2,3-dihydro-1,3-oxazine-2,4-dione, oxypyridine, aminopyridine, hydroxyquinoline, aminoquinoline, iso-carbostyryl, sulfonamide, 2H-1,3-benzothiazine-2,4-(3H)dione, benzotriazine, mercaptotriazole, dimercapto-tetrazapentalene, phthalic acid, naphthalic acid, phthalamine acid, a mixture of one or more of the above compounds with imidazole compounds, a mixture of at least one of phthalic acid, naphthalic acid or an acid anhydride thereof with phthalazine compounds, and a combination of phthalazine with maleic acid, itaconic acid, quinolinc acid and gentisinic acid. Further, there may also be effectively used those development accelerators described in Japanese Patent O.P.I. Publication Nos. 189628/1983 and 1934601/1983, which include, for example, 3-amino-5-mercaptop-1,2,4-triazole and 3-acylamino-5-mercaptop-1,2,4-triazole.

Those useful for the antifoggants are described in Japanese Patent Examined Publication No. 11113/1972, Japanese Patent O.P.I. Publication Nos. 90118/1974, 10724/1974, 97613/1974, 101019/1975, 130720/1974, 123331/1975, 47419/1976, 57435/1976, 78227/1976, 104338/1976, 19825/1978, 20923/1978, 50725/1976, 3223/1976, 42529/1976, 81124/1976, 51821/1979 and 93149/1980, British Pat. No. 1,455,271, U.S. Pat. Nos. 3,885,968, 3,700,457, 4,137,079 and 4,138,265, West German Patent No. 2,617,907. Examples of these antifoggants include, for example, mercuric salts, oxidizing agents such as N-halogenoacetamides, N-halogenosuccinimides, perchloric acid and the salts thereof, inorganic peroxides and peroxosulfate; acids and the salts thereof such as sulfonic acid, lithium laurate, rosin, diterpenic acid, thiosulfonic acid; sulfur-containing compounds such as mercapto compound-releasing compounds, thiouracil, disulfide, sulfur in the form of a simple substance, mercapto-1,2,4-triazole, thiazolinethione and polysulfide compounds; oxazoline; 1,2,4-triazole and phthalimide. Thiol compounds and more preferably thiophenol compounds described in Japanese Patent O.P.I. Publication No. 111636/1984 are also useful as the antifoggants.

As for the antifoggants, a hydroquinone derivative described in Japanese Patent Application No. 56506/1984, such as di-t-octyl hydroquinone, dodecanyl hydroquinone; and a combination of hydroquinone derivative and a benzotriazole derivative such as 4-sulfobenzotriazole and 5-carboxybenzotriazole described in Japanese Patent Application No. 66380/1984, are preferably used.

For the stabilizers, printout inhibitors especially for use after a heat-developing process may be used in combination. Examples thereof are given in Japanese Patent O.P.I. Publication Nos. 45228/1973, 119624/1975, 120328/1975, 46020/1978, which typically include halogenated hydrocarbons such as tetrabromobutane, tribromoethanol, 2-bromo-2-tolylacetamide, 2-bromo-2-tolylsulfonylacetamide, 2-tribromomethylsulfonylbenzothiazole and 2,4-bis(tribromomethyl)-6-methyltriazine.

Sulfur-containing compounds described in Japanese Patent Examined Publication No. 5393/1971, and Japanese Patent O.P.I. Publication Nos. 54329/1975 and 77034/1975 may be used for post-processing.

Further, they may contain the precursors of isothiuronium type stabilizers described in U.S. Pat. Nos. 3,301,678, 3,506,444, 3,824,103 and 3,844,788 and the precursors of activator stabilizers described in U.S. Pat. Nos. 3,669,670, 4,012,260 and 4,060,420.

Water releasing agents such as cane sugar and  $\text{NH}_4\text{Fe}(\text{SO}_4)_2 \cdot 12\text{H}_2\text{O}$  may also be used, and further, a heat-development may be carried out by supplying water as is described in Japanese Patent O.P.I. Publication No. 132332/1981.

To the heat-developable color photo-sensitive material of the invention, besides the constituents mentioned above, various additives and coating aids such as spectral sensitizing dyes, antihalation dyes, optical brightening agents, hardners, antistatic agents, plasticizers and spreading agents may be added if necessary.

It is preferred that the heat-developable color photo-sensitive materials of the invention is to contain in the same layer (1) a photo-sensitive silver halide, (2) a reducing agent, (3) a dye-providing material of the invention, (4) a binder, and, if required, (5) an organic silver salt. It is, however, not always needed to contain them into a single photographic component layer. For example, it is allowed that a photo-sensitive layer is divided into two layers and the components of the above-mentioned (1), (2), (4) and (5) are contained in one photo-sensitive layer, and the dye-providing material of the invention (3) is contained in the other layer which is provided adjacently to the one layer, provided that the reactions can be made with each other.

Further, the photo-sensitive layer may be separated into more than two layers, namely, a high-sensitive layer and a low-sensitive layer, and the like. The layer may be provided with one or more photo-sensitive layers which differ in color sensitivity. The layer may be provided with various photographic component layers such as an over layer, a subbing layer, a backing layer, an intermediate layer, or a filter layer.

In the same manner used for the preparation of heat-developable photo-sensitive materials of the invention, a coating solution is prepared each for a protective layer, an interlayer, a subbing layer, a backing layer and other photographic component layers and coated by such various coating methods as a dipping method, an air knife method, a curtain coating method, and a hopper coating method described in U.S. Pat. No. 3,681,294, thus the photo-sensitive materials are prepared.

If necessary, by the methods described in U.S. Pat. No. 2,761,791 and British Pat. No. 837,095, two or more layers can be simultaneously coated.

The constituents used for the photographic component layers of the heat-developable color photo-sensitive materials of the invention are coated on the support and the coating thickness after drying is preferably from 1 to 1,000  $\mu\text{m}$  and more preferably from 3 to 20  $\mu\text{m}$ .

The heat-developable color photo-sensitive material of the invention is color developed by being heated after imagewise exposure usually at from 80° C. to 200° C. and preferably at from 120° C. to 170° C. for from 1 sec. to 180 sec. and preferably from 1.5 sec. to 120 sec. And if necessary, it may be developed by contacting a water-impermeable material or it may be preheated at from 70° C. to 180° C. before exposure.

Various exposure means may be used for the heat-developable color photo-sensitive material of the invention. Latent images are obtained by imagewise exposure of rays of radiant light including visible radiation. Gen-

erally, light sources for ordinary color printing such as tungsten lamp, mercury lamp, xenon lamp, laser beam and CRT beam may be used as the light source thereof.

Heating methods applicable to ordinary heat-developable photo-sensitive materials may all be utilized, for example, bringing the materials into contact with a preheated block or plate, a heated roller or a heated drum, making the materials passing through high temperature atmosphere, using high-frequency heating, or providing a conductive layer in the photo-sensitive materials of the invention or in a thermal transfer image receiving layer (element) to utilize Joule's heat generated by applying electric current or a ferromagnetic field. Heating patterns have no particular limit, namely, it is allowed that the materials are preheated in advance and then heated again, that the materials are continuously heated by heating repeatedly for a short time at a high temperature and then for a long time at a low temperature, and that the materials are heated discontinuously, however, an easy heating pattern is most preferable. And it is also preferable that the exposure and the heating process are made simultaneously.

The image receiving member may be used for the invention provided that it is capable of receiving dyes released or formed by the heat development. It is preferred that the image receiving member is formed by the use of mordants used for the dye diffusion transfer type photo-sensitive material, or heat-resisting organic high molecular substance whose glass-transition temperature is not less than 40° C. and not more than 250° C.

Concrete examples of the above-mentioned mordants include secondary and tertiary amines containing nitrogen, heterocyclic compounds containing nitrogen and quaternary cationic compounds thereof; vinyl pyridine polymer and vinyl pyridinium cationic polymer described in U.S. Pat. Nos. 2,548,564, 2,484,430, 3,148,061 and 3,756,814; polymers containing dialkylamino group described in U.S. Pat. No. 2,675,316; aminoquanidine derivatives described in U.S. Pat. No. 2,882,156; reactive polymers of covalent bond type described in Japanese Patent O.P.I. Publication No. 137333/1979; mordants capable of cross-linking with gelatin and the like described in U.S. Pat. Nos. 3,625,694 and 3,859,096, and British Patent Nos. 1,277,453 and 2,011,012; aqueous sol type mordants described in U.S. Pat. Nos. 3,958,995, 2,721,852 and 2,798,063; water-insoluble mordants described in Japanese Patent O.P.I. Publication No. 61228/1975; various mordants described in U.S. Pat. No. 3,788,855, West German OLS Patent No. 2,843,320, Japanese Patent Nos. 30328/1978, 155528/1977, 125/1978, 1024/1978, 74430/1979, 124726/1979 and 22766/1980, U.S. Pat. Nos. 3,642,482, 3,488,706, 3,557,066, 3,271,147 and 3,271,148, Japanese Patent Examined Publication Nos. 29418/1980, 36414/1981 and 12139/1982, Research Disclosure 12045/1974.

An especially useful mordant is a polymer containing an ammonium salt, that is, a polymer containing quaternary amino group described in U.S. Pat. No. 3,709,690. A polymer containing an ammonium salt includes, for example, polystyrene-Co-N,N,N-tri-n-hexyl-N-vinylbenzylammonium chloride in which the ratio of styrene to vinylbenzylammonium chloride is from 1:4 to 4:1, preferably 1:1.

A typical image-receiving layer for a dye diffusion transfer is obtained by coating a mixture of a polymer containing an ammonium salt and gelatin.

The above-mentioned heat-resisting organic high molecular substances include polyacetals such as polystyrene whose molecular weight is from 2,000 to 85,000, a polystyrene derivative having a substituent in which carbon atoms are not more than four, polyvinyl cyclohexane, polyvinyl benzene, polyvinyl pyrrolidone, polyvinyl carbazole, polyallyl benzene, polyvinyl alcohol, polyvinyl formal, and polyvinyl butyral; polyesters such polyvinyl choride, chlorinated polyethylene, polyfluoroethylene trichloride, polyacrylonitrile, poly-N,N-dimethylacrylamide, a polyacrylate having p-cyanophenyl group, pentachlorophenyl group and 2,4-dichlorophenyl group, polyacrylicchloroacrylate, polymethylmethacrylate, polyethylmethacrylate, polypropylmethacrylate, polyisopropylmethacrylate, polyisobutylmethacrylate, poly-tert-butylmethacrylate, polycyclohexylmethacrylate, polyethylene glycol dimethacrylate, poly-2-cyano-ethylmethacrylate and polyethylene terephthalate; polycarbonates such as polysulfone, bisphenol A polycarbonate; polyanhydride, polyamides, cellulose acetates and the like. Synthetic polymers whose glass-transition temperature is not less than 40° C., which is described in Polymer Handbook 2nd ed. written by J. Brandrup and E. H. Immergut and published by John Wiley and Sons are also useful. These high molecular substance may be used independently or in combination with more than two, that is, as a copolymer.

Polymers particularly useful for the invention include cellulose acetate such as triacetate and diacetate; polyamides in combination with heptamethylenediamine and adipic acid, fluorenediisopropylamino and adipic acid, hexamethylenediamine and isophthalic acid, and the like; polyesters in combination with diethylene glycol and diphenyl carboxylic acid, bis-p-carboxyphenoxybutane and ethylene glycol, and the like; polyethylene terephthalate, polycarbonate and polyvinyl chloride. These polymers may be modified ones. For example, also useful are polyethylene terephthalate in which such modifiers as cyclohexane dimethanol, isophthalic acid, methoxypolyethylene glycol, 1,2-dicarbomethoxy-4-benzenesulfonic acid and the like. The layer containing polyvinyl chloride described in Japanese Patent Application No. 97907/1983 and the layer containing polycarbonate and a plasticizer are particularly preferable.

The above-mentioned polymers are used to form an image-receiving layer in the way that the polymer dissolved in a suitable solvent is coated onto a support; that a film-type image-receiving layer containing the polymer is laminated onto a support; or that a member containing the polymer, for example, a film may independently form an image-receiving layer (A layer for both an image-receiving layer and a support).

Further an image-receiving layer may be formed by providing an opaque layer (reflective layer) containing titanium oxide dispersed in gelatin on an image-receiving layer on a transparent support. When the opaque layer is provided, a transferred color image can be viewed in the form of a reflection type color image on the image-receiving layer from the side of the transparent support.

#### [EXAMPLES]

The examples of the invention will now be described below. It is, however, to be understood that the embodiments of the invention shall not be limited thereto.

## EXAMPLE-1

The dissolution of 620 mg of the exemplified dye-providing polymer (PY-1, Weight average molecular weight=11,500) was made in 2.1 ml of ethyl acetate. The resulted solution was mixed with an aqueous solution of 2.5% gelatin containing a surface active agent and added with water to make 6.5 ml. The resulted solution was then dispersed by means of a homogenizer so as to obtain a dispersed solution of the dye-providing polymer.

The above-mentioned 6.5 ml of dispersed solution were mixed up with polyvinyl pyrrolidone in an amount of 30,000 in average molecular weight, 0.2 ml of a 10% ethanol solution of guanidine trichloroacetate and 3.5 ml of water containing 500 mg of 1,5-pentanediol, and were added with 200 mg of the aforementioned reducing agent (R-3). After then, the pH value thereof was adjusted with 3% citric acid to 5.5. The resulted dispersed solution was added with silver iodobromide emulsion (containing 85 mg of gelatin) of 0.1  $\mu\text{m}$  in average grain size in an amount of  $1 \times 10^{-3}$  mole in terms of silver, and was added with water to make 15 ml. After then, the resulted solution was coated over to a polyethyleneterephthalate support by making use of a wire-bar so as to provide the light-sensitive layer of 8  $\mu\text{m}$  in thickness thereof on the support.

The obtained light-sensitive material was dried up and was then exposed to white light of 16,000 CMS through a step-wedge.

Next, an image receiving sheet was separately prepared by coating on a sheet of baryta paper polyvinyl chloride for the material of the image receiving layer thereof, and the image receiving layer surface and the coated surface of the aforementioned exposed light-sensitive material were attached to each other. After a thermal development was made at 155° C. for one minute, the image receiving sheet was peeled off, so that a transferred image in yellow was obtained on the image receiving sheet. Table-1 shows the maximum reflection density (Dmax) and the fog (Dmin) of the obtained transferred image.

## COMPARATIVE EXAMPLE-1

A light-sensitive material similar to that prepared in Example-1 was prepared in the same manner taken in the light-sensitive material of Example-1, except that the dye-providing polymer (PY-1) was replaced by the following comparative polymer A. The resulted comparative example was thermally developed in the same manner taken in Example-1. The results therefrom are shown in Table-1.

Comparative Polymer A

-continued



TABLE 1

| Dye-providing polymer |              | Reducing agent | D <sub>max</sub> | D <sub>min</sub> |
|-----------------------|--------------|----------------|------------------|------------------|
| Exemplification       | Amount added |                |                  |                  |
| Example 1             | PY-1         | 620 mg         | R-3              | 1.34             |
| Comparative           | Comparative  | 550 mg         | R-3              | 0.39             |
|                       | Polymer A    |                |                  | 0.15             |
|                       | Example 1    |                |                  |                  |

As is obvious from Table-1, in the thermally developable color light-sensitive materials not using any organic silver salt, it is understood that a D<sub>max</sub> of the sample using the dye-providing polymers of the invention is relatively greater and a D<sub>min</sub> thereof is relatively less than those of the comparative example.

## EXAMPLE-2

## [Preparation of 4-sulfobenzotriazole silver]

The dissolution of both 24 g of 4-sulfobenzotriazole and 4 g of sodium hydroxide was made by adding them into 300 ml of an ethanol-water mixed (1:1) solution. The resulted solution was added by dropping with 20 ml of a silver nitrate solution of 5 normality. At this time, a sodium hydroxide solution of 5 normality was also dropped thereinto at the same time, so as to keep the pH value of the solution from 7 to 8. After stirring the solution at room temperature for one hour, water was added to make 400 ml, so as to prepare a solution of 4-sulfobenzotriazole silver containing 20% excess amount of 4-sulfobenzotriazole.

## [Preparation of Light-sensitive Material]

A dissolution of both 620 mg of the dye-providing polymer (PY-1) similar to that used in Example-1 and 30 mg of 1,4-diethyl hydroquinone was made in 2.1 ml of ethyl acetate. The resulted solution was mixed up with 3 ml of a 2.5% gelatin solution containing a surface active agent and was added with water to make 6.5 ml. After then, the solution was dispersed by making use of a homogenizer, so that the dispersed solution of the dye-providing polymers was obtained. Next, 6 ml of the dispersed solution of the dye-providing polymers and 4 ml of the aforementioned 4-sulfobenzotriazole silver solution were mixed up and further 450 mg of polyvinyl pyrrolidone of 30,000 in average molecular weight, 120 mg of pentaerythritol, 420 mg of 1,5-pentanediol and 200 mg of the same reducing agent (R-3) as that used in Example-1 were added thereto. Then, the pH value thereof was adjusted to 5.5 with a 3% citric acid. The dispersed solution was added with a silver iodobromide emulsion having an average grain size of 0.05  $\mu\text{m}$  in an amount of  $3 \times 10^{-4}$  mole in terms of silver amount

(which contains 75 mg of gelatin), and was further added with water to make 14 ml. After then, the resulted matter was coated over to a polyethyleneterephthalate support to make the dried thickness thereof be 8  $\mu\text{m}$  by making use of a wire-bar, so that a light-sensitive layer was provided on the support.

After the resulted light-sensitive material was dried up, it was exposed to white-light of 32,000 CMS, through a step wedge. Then, an image-receiving sheet that was similar to that used in Example-1 was developed under the same conditions, so that a transferred image in yellow color was obtained on the image-receiving sheet. Table-2 shows the maximum reflection density (Dmax) and the fog (Dmin) of the obtained transferred image.

### EXAMPLE-3

A light-sensitive material similar to that obtained in Example-2 was prepared in the same manner as was taken in Example-2, except that the dye-providing polymer, PY-1, was replaced by the dye-providing polymers each shown in Table-2. The light-sensitive material thus prepared was thermally developed in the same manner as was taken in Example-2, and a transferred image in yellow color was obtained on an image receiving sheet. Table-2 also shows the results of the obtained transferred image density.

### EXAMPLE-4

A light-sensitive material similar to that obtained in Example 2 was prepared in the same manner as was taken in Example-2, except that the reducing agent was replaced by the reducing agents shown in Table-2, and the prepared light-sensitive materials were then exposed to light and thermally developed in the same manner as was taken in Example-2. Thereby, the transferred images in yellow color were obtained. Table-2 also shows the results of the transferred image density.

### COMPARATIVE EXAMPLE-2

A light-sensitive materials similar to that obtained in Example-2 were prepared in the same manner as was taken in Example-2, except that the dye-providing polymer, PY-1 was replaced by the aforementioned comparative polymer A and the following comparative polymer B, respectively. Thus prepared light-sensitive materials were thermally developed in the same manner as was taken in Example-2. Thereby, the transferred images in yellow color were obtained on an image-receiving sheet.

TABLE 2

|    |             | Dye-providing polymer |  | Amt added (mg) | Reducing agent | Dmax | Dmin |
|----|-------------|-----------------------|--|----------------|----------------|------|------|
|    |             | Exemplified No.       |  |                |                |      |      |
| 5  | Example 2   | PY-1<br>(Mw = 11,500) |  | 620            | R-3            | 1.84 | 0.08 |
| 10 | Example 3   | PY-1<br>(Mw = 10,900) |  | 500            | R-3            | 1.91 | 0.08 |
|    | Example 3   | PY-3<br>(Mw = 9,700)  |  | 400            | R-3            | 1.98 | 0.11 |
| 15 | Example 3   | PY-8<br>(Mw = 9,950)  |  | 480            | R-3            | 1.95 | 0.09 |
|    | Example 3   | PY-10<br>(Mw = 9,800) |  | 620            | R-3            | 1.79 | 0.07 |
| 20 | Example 4   | PY-1                  |  | 620            | R-1            | 1.80 | 0.11 |
|    | Example 4   | PY-1                  |  | 620            | R-9            | 1.72 | 0.06 |
|    | Comparative | Comparative polymer A |  | 550            | R-3            | 0.78 | 0.06 |
| 25 | Example 2   | Comparative Polymer B |  | 750            | R-3            | 1.23 | 0.09 |
|    | Example 2   |                       |  |                |                |      |      |

As is obvious from the results shown in Table-2, the thermally developable color light-sensitive materials of the invention are stable in the maximum reflection density at a substantially greater value and yellow transferred images in which fogs are further more improved can be obtained therefrom.

What is claimed is:

1. In a heat-developable color photo-sensitive material comprising a support bearing thereon a photographic component layer containing at least a photosensitive silver halide, a reducing agent, a binder and a dye-providing material; said heat-developable photosensitive material characterized in that at least one of said dye-providing materials is a polymer having a unit being derived from a monomer represented by the Formula [I] below;



wherein,  $\text{R}_1$  represents an alkyl group;  $\text{R}_2$  represents an alkyl or an aryl group;  $\text{R}_3$  represents a divalent hydrocarbon;  $\text{R}_4$  represents an alkyl group or a hydrogen

### Comparative Polymer B



( $\text{x} = 50$  weight %)  
( $\text{y} = 50$  weight %)  
(Mw = 10,500)

atom; J represents a divalent bonded group; l is an integer of 0 or 1; and m is an integer of 0 or 1.

2. The heat-developable color photo-sensitive material as claimed in claim 1, wherein the weight average molecular weight of said polymer is from 1,500 to 100,000.

3. The heat-developable color photo-sensitive material as claimed in claim 1, wherein the molecular weight of the residual group



having the Formula [I] is not more than 700.

4. The heat-developable color photo-sensitive material as claimed in claim 1, wherein  $\text{R}_4$  in the Formula [I] representing said monomer is an alkyl group having not more than four carbon atoms.

5. The heat-developable color photo-sensitive material as claimed in claim 1, wherein  $\text{R}_2$  in the Formula [I] representing said monomer is a phenyl group.

6. The heat-developable color photo-sensitive material as claimed in claim 1, wherein J in the Formula [I] representing said monomer is  $-\text{NHCO}-$  or  $-\text{OCO}-$ .

7. The heat-developable color photo-sensitive material as claimed in claim 1, wherein said binder comprises, in combination, gelatin and/or the derivative thereof and polyvinyl pyrrolidone or polyvinyl alcohol.

8. The heat-developable color photo-sensitive material as claimed in claim 7, wherein said polyvinyl pyrrolidone is from 1,000 to 400,000 in molecular weight.

9. The heat-developable color photo-sensitive material as claimed in claim 1, wherein said polymer is a copolymer having at least one kind of the monomers each having the Formula [I].

5

10

15

30

35

10. The heat-developable color photo-sensitive material as claimed in claim 9, wherein said unit derived from the monomer having the Formula [I] is from 10 to 90% by weight of the copolymer.

11. The heat-developable color photo-sensitive material as claimed in claim 1, wherein said reducing agent is represented by the Formula [II] below;



wherein,  $\text{R}_5$  and  $\text{R}_6$  each represent hydrogen or an alkyl group which is allowed to have a substituent and has one to 30 carbon atoms, and the  $\text{R}_5$  and  $\text{R}_6$  are also allowed to close a ring so as to form a heterocyclic ring;  $\text{R}_7$ ,  $\text{R}_8$ ,  $\text{R}_9$  and  $\text{R}_{10}$  each represent hydrogen, a halogen, a hydroxy group, an amino group, an alkoxy group, an acylamide group, a sulfonamide group, an alkylsulfonamide group, or an alkyl group which is allowed to have a substituent and has one to 30 carbon atoms; and the  $\text{R}_7$  and  $\text{R}_5$ , and the  $\text{R}_9$  and  $\text{R}_6$  each are allowed to close a ring so as to form a heterocyclic ring, respectively; and M represents an alkaline metal atom or a compound containing an ammonium group, a nitrogen-containing organic base or a quaternary nitrogen atom.

12. The heat-developable color photo-sensitive material as claimed in claim 11, wherein at least one of  $\text{R}_5$  and  $\text{R}_6$  is an alkyl having one to four carbon atoms and wherein the alkyl group for  $\text{R}_7$ ,  $\text{R}_8$ ,  $\text{R}_9$  and  $\text{R}_{10}$  contains one to four carbon atoms.

\* \* \* \* \*

40

45

50

55

60

65